

## UNITED STATES PATENT OFFICE

2,045,052

## PAPER MANUFACTURE

Harold Robert Rafton, Andover, Mass., assignor  
to Raffold Process Corporation, a corporation  
of Massachusetts

No Drawing. Application May 5, 1932,  
Serial No. 609,555

32 Claims. (Cl. 91—68)

This invention relates to the production of sized paper filled with alkaline filler.

The principal object of this invention is to produce sized paper filled with alkaline filler in which the sizing is applied to the paper web.

A further object is to avoid the necessity for the heating of the paper web to a temperature sufficient to flux any thermoplastic material employed as sizing agent.

A further object is the production of sized paper filled with alkaline filler by the application of non-thermoplastic sizing agent to the paper web.

A further object is the application of the sizing agent to the paper web in solution form, particularly in solution in an organic solvent.

Other objects and advantages of this invention will become apparent during the course of the following description.

In my copending application Serial No. 487,377, filed October 8, 1930, of which the present application is a continuation in part, I have described a method whereby paper filled with alkaline filler may be sized by the application of thermoplastic material, such as paraffin, in liquid association to a paper web containing alkaline filler. By "liquid association" I mean that the thermoplastic material is present as such either in the form of an emulsion or solution. In the case of emulsions, or solutions in water-miscible solvents, the application is made either to the wet or to the already substantially dried web; in the case of solutions made with solvents immiscible with water, application is made only to the already substantially dried web. After the evaporation of the liquid, a sized web results. In order to secure uniformity of sizing, the web is raised to a temperature sufficiently high to flux the thermoplastic material.

Further development of the above process has shown that sized paper filled with alkaline filler in which the sizing is substantially uniform may be produced even when the paper web is not subjected to a temperature sufficiently high to flux the thermoplastic material. This has been found to be particularly so in certain cases where solutions of thermoplastic material in a solvent are employed. The necessity of subjecting the web to such fluxing temperature appears to depend among other things somewhat upon the nature of the solvent employed but chiefly upon the nature of the thermoplastic material used. Certain solvents appear to have the property of effecting more uniform distribution of the thermoplastic material in the web, and likewise cer-

tain thermoplastic materials seem to distribute themselves more uniformly in the web than do others even when the same solvent is employed. Although I do not wish to be limited by any generalization, I have noted that apparently certain materials of a waxy nature seem to have their sizing distribution in the web improved by fluxing, whereas certain materials of a resinous nature seem to distribute themselves substantially uniformly in the web when in solution and do not appear to need fluxing.

The latter condition appears to be true where a resin such as rosin is used in solution in a solvent, in which case only enough heat may be supplied to the web to evaporate the solvent without it being necessary to actually raise the temperature of the web to the fluxing or so-called "sintering" temperature of the rosin. Of course if such temperature should be reached, this is usually not objectionable; but as such temperature is not ordinarily reached in the evaporation of low boiling point organic solvents such as may conveniently be used in the practice of my process, and particularly where the solvent is evaporated under reduced pressure, it is not necessary simultaneously or subsequently to supply the necessary heat so that the web will reach such temperature. Any one of a number of solvents may be used, among which the chlorinated hydrocarbons such as carbon tetrachloride, ethylene dichloride, and the like, may be recommended as being particularly satisfactory.

In the preferred practice of my invention a web containing alkaline filler is formed, for example by feeding to the web-forming device of a paper machine a fibrous mix in which alkaline filler is present. To this web a solution of thermoplastic material in a solvent, for example rosin in ethylene dichloride, is applied. The liquid content of the web is then evaporated and a sized paper web filled with alkaline filler results. The point of application, the method of application, the concentration and amount of thermoplastic material to be applied, and other necessary or optional details of my process, are similar in general to those employed in my above referred to copending application, but for the sake of completeness will be fully set forth immediately below together with certain other features which I have found desirable.

The thermoplastic material may be applied in a solvent, which is usually organic, as the thermoplastic materials I employ are normally substantially insoluble in water. If the material be applied in a water-miscible organic solvent, such

5

15

20

25

30

35

40

45

50

55

- for example as ethyl alcohol, it may be applied at any convenient point on the paper machine either where the web is still in wet condition, for example at or just after the press rolls, or at a 5 point where water has been substantially removed from the web, for example preferably just after the driers; or the solution of the material may optionally be applied to the paper web subsequent to the paper machine by a separate process.
- 10 In the case where a water-miscible solvent is employed and the solution is applied to the wet web, the wet web may then be dried as usual, and in the interest of economy suitable means should be provided for recovery of the solvent from the 15 evaporated liquid. In the case of application of a solution containing such solvent to a dried web, provision must be made for subsequent removal of the solvent from the web, for example by passage of the web over driers or by festooning in a 20 hot atmosphere, or the like. In any case, in the interest of economy, suitable solvent recovery means should be provided.

In the case of the use of a solution of thermoplastic material in a solvent substantially immiscible with water, and this is the type of solvent which I find it most convenient to employ, it is not suitable to apply such a solution to the wet web but it should be applied rather to the web after the web has been substantially deprived of 30 its water, preferably subsequent to the paper machine driers and conveniently before the calenders, and then provision must be made for removing the solvent such as by passage of the web over driers or through a hot atmosphere, with suitable 35 provision for recovering the solvent. However, in some cases the application of the solution of the thermoplastic material may take place as an independent process subsequent to the paper machine operation, suitably by a coating or saturating machine in which means is provided for subsequent removal and recovery of the solvent.

The solution of the thermoplastic material may be applied to the web by any of the various methods for applying liquids to a paper web, such as 45 by passing the web through a trough or vat containing the solution, or by applying the solution by a brush, for example by a rotary brush, or by a contact roll or rolls, or by spraying or the like, or in the case of water miscible solvents by a supply box at one or more of the press rolls. The 50 method of application employed in any given instance is that which is best adapted for use at the particular point at which the solution is applied and should be chosen with regard to the 55 particular conditions to be met in any given case, all of which will be apparent to one skilled in the art. For example, I have found that the application by a trough followed by a pair of squeeze rolls is a convenient method of application, especially 60 for use with solutions in water-immiscible solvents which are applied to the dry web.

The concentration of the solutions used depends to a certain extent upon the method of employing them and the point of application. For application 65 by a roll, the solutions may in general be more concentrated, but for immersion or spraying it is more suitable to have them relatively dilute. An example of a suitable solution concentration to be applied by a contact roll is 10 per cent. 70 of thermoplastic material by weight, whereas for applying by a trough a 5 per cent. concentration by weight is suitable. I do not, however, limit myself to these concentrations and they may be widely varied according to circumstances as indicated 75 above and still produce satisfactory results.

The amount of thermoplastic material required for sizing varies somewhat as will be apparent, with the grade of paper made, its fibrous constituents, the percentage of filler, and the like, but in general the amount used will vary from under 1 per cent. up to several per cent. or more, calculated as the weight of thermoplastic material on the weight of paper. Naturally when very small amounts are applied the sizing effect imparted will be slight, however, two per cent. will usually 1 impart a satisfactory degree of sizing and, in any event, this is a convenient percentage to try in the first place when tentatively adjusting the amount of thermoplastic material to be applied.

As the solution of the thermoplastic material is 1 preferably applied continuously to the web, suitable means such as a pump should be employed for supplying the agent to the applying device, and the amount of agent applied should preferably vary regularly with the paper machine speed and 2 be adjustable to the various grades and weights of paper run. Other things being equal, after proper 2 adjustments are made, the amount of thermoplastic material applied may perhaps be most conveniently regulated by regulating the concentra- 2 tion of the solution employed.

In the case of a solution of thermoplastic material in a water-miscible solvent applied to a wet web, the evaporation of the solvent and the associated water is suitably accomplished by the application to the paper web of heat or reduced pressure or both such, for example, as on the ordinary paper machine drier or in a vacuum drier, in either case with suitable means for the recovery of the solvent. Where the solution is applied to 3 the already substantially dried web, such as may be the case when a water-miscible solvent, and must be the case when a water-immiscible solvent, is employed, there is not present any substantial amount of moisture and thus the means 4 for evaporation of the solvent from the web as well as the recovery means are somewhat simplified. Moreover, the amount of heat required for the evaporation of the solvent over that for the joint evaporation of solvent and water is considerably less and thus smaller drying capacity is necessary. In this case, as in the case of the wet web application mentioned above, the evaporation of the solvent is suitably accomplished by the application to the paper web of heat or reduced pressure or both. An evacuated chamber such as a 5 vacuum drier or the like may be employed, operated as part of the paper machine equipment or as a separate unit. Or my process may be carried out with less capital expenditure by means of solvent evaporating apparatus operated in an enclosure which is maintained at substantially atmospheric pressure or just slightly below. A suitable apparatus for this purpose is described in my copending application Serial No. 640,714, filed Nov. 1, 1932. Such apparatus may be operated as part of the paper machine equipment or as a separate step after the paper machine.

Whether atmospheric pressure or vacuum solvent evaporating apparatus be used suitable solvent recovery means should of course also be provided.

By my improved method of applying thermoplastic material to the paper web, I have been able to make satisfactorily sized alkaline filled papers without the necessity of fluxing the material in the paper web after application. The paper made is what is known as sized paper, i. e. resistant to aqueous writing ink in varying degree according to the degree of sizing desired,

and is similar in appearance to and by ordinary observation cannot be readily distinguished from ordinary sized paper hitherto made by other means, for example, from clay filled paper sized by the ordinary method of resin sizing in the beater. Of course if larger amounts of thermoplastic material are employed, the sized paper produced assumes more marked waterproof characteristics. The sized paper I refer to is not to be confused with paper, such as waxed paper or the like, which is saturated or substantially saturated with the sizing agent in question; and where the term "sized paper" is employed herein it is used in the sense in which it is ordinarily used in the paper industry as indicated in the definition thereof given above and is intended to exclude paper which is saturated or substantially saturated with the sizing agent in question. And where in the claims I speak of "applying" sizing agent in a solvent, as to a fibrous web, or "distributing" it therein, I mean that the quantity of such sizing agent so applied or distributed shall be insufficient to result in the production of paper saturated or substantially saturated with the sizing agent in question. It is to be understood that such "sized" paper as described herein is distinct from the so-called "surface-sized" or "coated" paper which is produced by applying animal or similar substantially water soluble size or a coating of similar nature to a paper web, either on the paper machine or subsequently by a separate process.

It is possible to employ my sizing method for applying additional sizing to a web containing alkaline filler, which web is already partially sized by other methods, and such use of my process falls within the scope of my invention.

One advantage of my present improved process is that it simplifies my former process, and requires less heat for carrying it out. Another advantage is that it now opens up the possibility of using other sizing agents by this method which materials in themselves are not thermoplastic or, if thermoplastic do not flux readily at temperatures ordinarily employed in paper manufacture. Materials of the latter type are for example cellulose compounds or derivatives, for example esters such as cellulose acetate, nitrate or the like, and these as well as the non-thermoplastic materials may be dissolved in suitable solvents such as organic solvents, applied to the paper web, and the solvent evaporated. Uniform sizing throughout the sheet is thus obtained despite the fact that the material itself is substantially non-fluxible or not readily fluxible at least at the temperature employed.

It is to be understood that I may if I desire actually apply heat to the sized substantially solvent-free web, providing that such heat is not sufficient substantially to flux the sizing agent employed.

In place of resins other thermoplastic materials may be used such as gums or the like, including synthetic thermoplastics such as obtained for example by chemical condensation. In the case of non-thermoplastic sizing agents, I may use any such, including synthetic non-thermoplastic materials, such as for example as those obtained by chemical condensation. Non-thermoplastic materials are well known in the art, specific examples being the product formed on standing from beta-elaeostearin, such as referred to in Thorpe, "Dictionary of Applied Chemistry", Vol. VII, Longmans, Green & Co.,

New York, 1927, page 227, last full sentence at bottom of second column; and infusible resins, such for example as the Baekeland infusible resin, referred to in Ellis, "Synthetic Resins and Their Plastics", The Chemical Catalogue Co. Inc., N. Y., 1923, page 126, last paragraph. Also I may employ mixtures of thermoplastic and non-thermoplastic material if desired; and in certain cases mixtures of other material with either thermoplastic or non-thermoplastic material, said other material serving to modify the characteristics of said thermoplastic or non-thermoplastic material in known manner, such as in respect to plasticity, thermoplasticity, solubility, chemical composition and the like. Whereas I may use either thermoplastic or non-thermoplastic sizing agents substantially inert to alkali, this is not necessary as the agents I use may be reactive with alkali. In the latter case where such agents in the broke from my sized paper filled with alkaline filler are reintroduced in the beater, they may tend to react with the alkaline filler to cause foam, which however, can be controlled by suitable means such, for example, as by the addition of acidic material such as alum at the dilute stage of the papermaking process as has already been disclosed in one or more of my issued patents.

It is to be understood, however, in respect to sizing agents which are saponifiable, such for example as rosin, that such sizing agents are to be used only in the substantially unsaponified condition. Thus, when material reactive with alkali, such as saponifiable material, is stated to be dissolved in solvent, its presence therein is intended to be confined to that condition in which it is substantially unreacted upon by alkali.

Where I speak of "synthetic thermoplastic material such as obtained by chemical condensation" (an example of which is the condensation of an aldehyde with a phenol), I mean to include material originally liquid or thermoplastic which may eventually become non-thermoplastic after application to the web.

Where I speak of "sizing agents" herein, such as for example either thermoplastic or non-thermoplastic material, I mean to confine said agents to material which is substantially insoluble in water. Inasmuch as the sizing agents I employ are thus substantially water insoluble, naturally where I used the word "solvent" in connection with these materials, I mean to confine myself to solvents other than water which are liquid in use, although of course for example with certain water miscible solvents such as ethyl alcohol there may be present at times in the solvent used a certain amount of water, which water however does not act in the present instance as a solvent.

In connection with the term "solvent", it is obvious that if there should be employed material of such low vapor pressure, that is to say such high boiling point, that the substantial removal of the solvent would necessitate operating at temperatures sufficiently high to substantially injure the web, the resulting process would not be operative for the intended purpose. Therefore, I disclaim the use of solvents except those having sufficiently high vapor pressure, that is to say sufficiently low boiling point, that they may be substantially removed from the web for example by at least one of the herein described procedures at a temperature which will not be sufficiently high to substantially injure the web.

By the term "alkaline filler" I mean substantially water insoluble filler which when agitated in contact with freshly boiled distilled water, say for an hour, will impart a pH value to such water greater than 7.0, that is, which will be on the alkaline side of the neutral point. Among fillers in this group may be mentioned calcium carbonate, of which lime mud from the causticizing process is one form; calcium carbonate magnesium basic carbonate employed in the paper disclosed in my United States Patent No. 1,595,416, issued August 10, 1926; calcium carbonate magnesium hydroxide disclosed in my United States Patent No. 1,415,391, issued May 9, 1922; and other substantially water insoluble normal or basic carbonates of alkaline earth metals, (which expression is herein intended to include magnesium), or compounds, double salts, or other physically associated mixtures of these with one or more other acid soluble materials of a substantially water insoluble nature. By the term "alkaline filler" I also intend to include fibrous material and/or other material such as paper coating constituents or the like containing one or more compounds of the character referred to, such as "old papers" or similar papers, "broke", or the like.

When I use the word "paper" herein, I use it in the broad sense to include products of manufacture of all types and of all weights and thicknesses, which contain as an essential constituent a considerable amount of prepared fibre and which are capable of being produced on a Fourdrinier, cylinder, or other forming, felting, shaping or molding machine.

While I have described in detail the preferred embodiment of my invention, it is to be understood that the details of procedure, the proportions of ingredients, and the arrangement of steps may be widely varied without departing from the spirit of the invention or the scope of the subjoined claims.

I claim:

1. The method of manufacturing sized paper filled with alkaline filler comprising preparing a fibrous web containing alkaline filler, applying to said web substantially water insoluble sizing agent dissolved in a solvent therefor, said sizing agent in such solution being characterized by being capable of distributing itself in said web to impart a substantially uniform sizing effect thereto at a temperature at which no substantial fluxing of said sizing agent occurs, said sizing agent in such solution being further characterized by being substantially unreacted upon by alkali, and evaporating substantially completely the liquid content of said web, but without bringing about any substantial fluxing of said sizing agent in said web, said sizing agent applied to said web being sufficient in amount to impart sizing effect to said paper.

2. The method of manufacturing sized paper filled with alkaline filler comprising preparing a fibrous web containing alkaline filler, applying to said web substantially water insoluble sizing agent dissolved in a solvent therefor, said sizing agent in such solution being characterized by being capable of distributing itself in said web to impart a substantially uniform sizing effect thereto at a temperature at which no substantial fluxing of said sizing agent occurs, said sizing agent in such solution being further characterized by being substantially unreacted upon by alkali, and evaporating substantially completely the liquid content of said web by means of reduced pressure and heat, said heat being insufficient to bring about any substantial fluxing of said sizing agent in said web, said sizing agent applied to said web being sufficient in amount to impart sizing effect to said paper.

3. The method of manufacturing sized paper filled with alkaline filler comprising preparing a fibrous web containing alkaline filler, substantially drying said web, applying to said substantially dry web substantially water insoluble sizing agent dissolved in a solvent therefor, said sizing agent in such solution being characterized by being capable of distributing itself in said web to impart a substantially uniform sizing effect thereto at a temperature at which no substantial fluxing of said sizing agent occurs, said sizing agent in such solution being further characterized by being substantially unreacted upon by alkali, and evaporating substantially completely said solvent content of said web, but without bringing about any substantial fluxing of said sizing agent in said web, said sizing agent applied to said web being sufficient in amount to impart sizing effect to said paper.

4. The method of manufacturing sized paper filled with alkaline filler comprising preparing a fibrous web containing alkaline filler, substantially drying said web, applying to said substantially dry web substantially water insoluble sizing agent dissolved in a solvent therefor, said sizing agent in such solution being characterized by being capable of distributing itself in said web to impart a substantially uniform sizing effect thereto at a temperature at which no substantial fluxing of said sizing agent occurs, said sizing agent in such solution being further characterized by being substantially unreacted upon by alkali, and evaporating substantially completely said solvent content of said web by means of reduced pressure and heat, said heat being insufficient to bring about any substantial fluxing of said sizing agent in said web, said sizing agent applied to said web being sufficient in amount to impart sizing effect to said paper.

5. The method of manufacturing sized paper filled with alkaline filler comprising preparing a fibrous web containing alkaline filler, substantially drying said web, applying to said substantially dry web substantially water insoluble sizing agent dissolved in a solvent therefor, said sizing agent in such solution being characterized by being capable of distributing itself in said web to impart a substantially uniform sizing effect thereto at a temperature at which no substantial fluxing of said sizing agent occurs, said sizing agent in such solution being further characterized by being substantially unreacted upon by alkali, and evaporating substantially completely said solvent content of said web by means of reduced pressure and heat, said heat being insufficient to bring about any substantial fluxing of said sizing agent in said web, said sizing agent applied to said web being sufficient in amount to impart sizing effect to said paper.

6. The method of manufacturing sized paper filled with alkaline filler comprising preparing a fibrous web containing alkaline filler, substantially drying said web, applying to said substantially dry web substantially water insoluble sizing agent dissolved in organic solvent, said sizing agent in such solution being characterized by being capable of distributing itself in said web to impart a substantially uniform sizing effect thereto at a temperature at which no substantial fluxing of said sizing agent occurs, said sizing agent in such solution being further characterized by being substantially unreacted upon by alkali, and evaporating substantially completely said organic solvent content of said web by means of heat, said heat being insufficient to bring about any substantial fluxing of said sizing agent in said web, said sizing agent applied to said web being sufficient in amount to impart sizing effect to said paper.

7. The steps in a method of manufacturing sized paper filled with alkaline filler comprising distributing substantially water insoluble sizing agent in a fibrous web containing alkaline filler by means of a vehicle comprising organic solvent in which said sizing agent is soluble, said sizing agent being characterized by being capable of distributing itself by means of said vehicle in said web to impart a substantially uniform sizing effect thereto at a temperature at which no substantial fluxing of said sizing agent occurs, said

- sizing agent being further characterized by being in a condition in which it is substantially unreacted upon by alkali, and evaporating substantially completely said organic solvent content of 5 said web, but without bringing about any substantial fluxing of said sizing agent in said web, said sizing agent distributed in said web being sufficient in amount to impart sizing effect to said paper.
- 10 7. The method of manufacturing sized paper filled with alkaline filler comprising preparing a fibrous web containing alkaline filler, applying to said web substantially water insoluble sizing agent comprising thermoplastic material dissolved 10 in a solvent therefor, said sizing agent in such solution being characterized by being capable of distributing itself in said web to impart a substantially uniform sizing effect thereto at a temperature at which no substantial fluxing of said sizing agent occurs, and evaporating substantially completely 15 the liquid content of said web, but without bringing about any substantial fluxing of said thermoplastic material in said web, said sizing agent applied to said web being sufficient in amount to impart sizing effect to said paper.
- 20 8. The method of manufacturing sized paper filled with alkaline filler comprising preparing a fibrous web containing alkaline filler, applying to said web substantially water insoluble sizing agent 20 comprising thermoplastic material dissolved in a solvent therefor, said sizing agent in such solution being characterized by being capable of distributing itself in said web to impart a substantially uniform sizing effect thereto at a temperature at which no substantial fluxing of said sizing agent occurs, and evaporating substantially completely 25 the liquid content of said web by means of reduced pressure and heat, said heat being insufficient to bring about any substantial fluxing of said thermoplastic material in said web, said sizing agent applied to said web being sufficient in amount to impart sizing effect to said paper.
- 30 9. The method of manufacturing sized paper filled with alkaline filler comprising preparing a fibrous web containing alkaline filler, substantially 30 drying said web, applying to said substantially dry web substantially water insoluble sizing agent comprising thermoplastic material dissolved in a solvent therefor, said sizing agent in such solution being characterized by being capable of distributing itself in said web to impart a substantially uniform sizing effect thereto at a temperature at which no substantial fluxing of said sizing agent occurs, and evaporating substantially completely 35 the liquid content of said web, but without bringing about any substantial fluxing of said thermoplastic material in said web, said sizing agent applied to said web being sufficient in amount to impart sizing effect to said paper.
- 40 10. The method of manufacturing sized paper filled with alkaline filler comprising preparing a fibrous web containing alkaline filler, substantially 40 drying said web, applying to said substantially dry web substantially water insoluble sizing agent comprising thermoplastic material dissolved in a solvent therefor, and evaporating substantially completely 45 the liquid content of said web, but without bringing about any substantial fluxing of said rosin in said web, said sizing agent applied to said web being sufficient in amount to impart sizing effect to said paper.
- 50 11. The method of manufacturing sized paper filled with alkaline filler comprising preparing a fibrous web containing alkaline filler, substantially 50 drying said web, applying to said substantially dry web substantially water insoluble sizing agent comprising thermoplastic material dissolved in a solvent therefor, and evaporating substantially completely 55 the liquid content of said web by means of reduced pressure and heat, said heat being insufficient to bring about any substantial fluxing of said rosin in said web, said sizing agent applied to said web being sufficient in amount to impart sizing effect to said paper.
- 60 12. The method of manufacturing sized paper filled with alkaline filler comprising preparing a fibrous web containing alkaline filler, substantially 60 drying said web, applying to said substantially dry web substantially water insoluble sizing agent comprising thermoplastic material dissolved in a solvent therefor, and evaporating substantially completely 65 the liquid content of said web by means of reduced pressure and heat, said heat being insufficient to bring about any substantial fluxing of said rosin in said web, said sizing agent applied to said web being sufficient in amount to impart sizing effect to said paper.
- 70 13. The method of manufacturing sized paper filled with alkaline filler comprising preparing a fibrous web containing alkaline filler, applying to said web substantially water insoluble sizing agent comprising rosin dissolved in a solvent therefor, and evaporating substantially completely 70 the liquid content of said web, but without bringing about any substantial fluxing of said rosin in said web, said sizing agent applied to said web being sufficient in amount to impart sizing effect to said paper.
- 75 14. The method of manufacturing sized paper filled with alkaline filler comprising preparing a fibrous web containing alkaline filler, applying to said web substantially water insoluble sizing agent comprising rosin dissolved in a solvent therefor, and evaporating substantially completely 75 the liquid content of said web by means of reduced pressure and heat, said heat being insufficient to bring about any substantial fluxing of said rosin in said web, said sizing agent applied to said web being sufficient in amount to impart sizing effect to said paper.
- 80 15. The method of manufacturing sized paper filled with alkaline filler comprising preparing a fibrous web containing alkaline filler, substantially 80 drying said web, applying to said substantially dry web substantially water insoluble sizing agent comprising rosin dissolved in a solvent therefor, and evaporating substantially completely 85 the liquid content of said web, but without bringing about any substantial fluxing of said rosin in said web, said sizing agent applied to said web being sufficient in amount to impart sizing effect to said paper.

16. The method of manufacturing sized paper filled with alkaline filler comprising preparing a fibrous web containing alkaline filler, substantially drying said web, applying to said substantially dry web substantially water insoluble sizing agent comprising rosin dissolved in a solvent therefor, and evaporating substantially completely said solvent content of said web by means of reduced pressure and heat, said heat being insufficient to bring about any substantial fluxing of said rosin in said web, said sizing agent applied to said web being sufficient in amount to impart sizing effect to said paper.
17. The method of manufacturing sized paper filled with alkaline filler comprising preparing a fibrous web containing alkaline filler, substantially drying said web, applying to said substantially dry web substantially water insoluble sizing agent comprising rosin dissolved in organic solvent, and evaporating substantially completely said organic solvent content of said web by means of heat, said heat being insufficient to bring about any substantial fluxing of said rosin in said web, said sizing agent applied to said web being sufficient in amount to impart sizing effect to said paper.
18. The method of manufacturing sized paper filled with alkaline filler comprising preparing a fibrous web containing alkaline filler, substantially drying said web, applying to said substantially dry web substantially water insoluble sizing agent comprising rosin dissolved in organic solvent, and evaporating substantially completely said organic solvent content of said web by means of reduced pressure and heat, said heat being insufficient to bring about any substantial fluxing of said rosin in said web, said sizing agent applied to said web being sufficient in amount to impart sizing effect to said paper.
19. The method of manufacturing sized paper filled with alkaline filler comprising preparing a fibrous web containing alkaline filler, applying to said web substantially water insoluble sizing agent comprising non-thermoplastic material dissolved in a solvent therefor, said sizing agent in such solution being characterized by being substantially unreacted upon by alkali, and evaporating substantially completely the liquid content of said web, said sizing agent applied to said web being sufficient in amount to impart sizing effect to said paper.
20. The method of manufacturing sized paper filled with alkaline filler comprising preparing a fibrous web containing alkaline filler, applying to said web substantially water insoluble sizing agent comprising non-thermoplastic material dissolved in a solvent therefor, said sizing agent in such solution being characterized by being substantially unreacted upon by alkali, and evaporating substantially completely the liquid content of said web by means of reduced pressure and heat, said sizing agent applied to said web being sufficient in amount to impart sizing effect to said paper.
21. The method of manufacturing sized paper filled with alkaline filler comprising preparing a fibrous web containing alkaline filler, substantially drying said web, applying to said substantially dry web substantially water insoluble sizing agent comprising non-thermoplastic material dissolved in a solvent therefor, said sizing agent in such solution being characterized by being substantially unreacted upon by alkali, and evaporating substantially completely said solvent content of said web by means of heat, said sizing

- agent applied to said web being sufficient in amount to impart sizing effect to said paper.
22. The method of manufacturing sized paper filled with alkaline filler, comprising preparing a fibrous web containing alkaline filler, substantially drying said web, applying to said substantially dry web substantially water insoluble sizing agent comprising non-thermoplastic material dissolved in a solvent therefor, said sizing agent in such solution being characterized by being substantially unreacted upon by alkali, and evaporating substantially completely said solvent content of said web by means of reduced pressure and heat, said sizing agent applied to said web being sufficient in amount to impart sizing effect to said paper.
23. The method of manufacturing sized paper filled with alkaline filler comprising preparing a fibrous web containing alkaline filler, substantially drying said web, applying to said substantially dry web substantially water insoluble sizing agent comprising non-thermoplastic material dissolved in organic solvent, said sizing agent in such solution being characterized by being substantially unreacted upon by alkali, and evaporating substantially completely said organic solvent content of said web by means of heat, said sizing agent applied to said web being sufficient in amount to impart sizing effect to said paper.
24. The steps in a method of manufacturing sized paper filled with alkaline filler comprising distributing substantially water insoluble sizing agent comprising non-thermoplastic material in a fibrous web containing alkaline filler by means of a vehicle comprising organic solvent in which said sizing agent is soluble, said sizing agent being characterized by being in a condition in which it is substantially unreacted upon by alkali, and evaporating substantially completely said organic solvent content of said web, said sizing agent distributed in said web being sufficient in amount to impart sizing effect to said paper.
25. Sized filled paper comprising fibrous material, alkaline filler, and sizing comprising substantially water insoluble cellulose derivative deposited out of a solution thereof in a solvent.
26. Sized filled paper comprising fibrous material, alkaline filler, and cellulose ester deposited out of a solution thereof in a solvent.
27. Sized filled paper comprising fibrous material, alkaline filler, and sizing comprising substantially water insoluble non-thermoplastic material substantially unreactive with alkali.
28. Sized filled paper comprising fibrous material, alkaline filler, and sizing comprising synthetic substantially water insoluble non-thermoplastic material substantially unreactive with alkali.
29. Sized filled paper resulting from applying to a fibrous web containing alkaline filler substantially water insoluble sizing agent dissolved in a solvent therefor, said sizing agent in such solution being characterized by being capable of distributing itself in said web to impart a substantially uniform sizing effect thereto at a temperature at which no substantial fluxing of said sizing agent occurs, said sizing agent in such solution being further characterized by being substantially unreacted upon by alkali, and subsequently substantially removing said solvent from said web, but without bringing about any substantial fluxing of said sizing agent in said web, said sizing agent applied to said web being sufficient in amount to impart sizing effect to said paper.

30. Sized filled paper resulting from distributing substantially water insoluble sizing agent which comprises non-thermoplastic material in a condition in which it is substantially unreacted upon by alkali in a fibrous web containing alkaline filler by means of a vehicle comprising a solvent in which said sizing agent is soluble, and subsequently substantially removing said solvent from said web, said sizing agent distributed in said web being sufficient in amount to impart sizing effect to said paper.

31. Paper filled with alkaline filler comprising fibrous material, alkaline filler, and substantially water insoluble sizing agent, said sizing agent having been provided by deposition out of solution thereof in an organic solvent by substantially completely removing said solvent by evaporation, said sizing agent in such solution being characterized by being substantially unreacted upon

by alkali, said sizing agent being further characterized by being capable of imparting a substantially uniform sizing effect at a temperature at which no substantial fluxing of said sizing agent occurs.

32. Paper filled with alkaline filler comprising fibrous material, alkaline filler, sizing, and, additionally, substantially water insoluble sizing agent, said sizing agent having been provided by deposition out of solution thereof in an organic solvent by substantially completely removing said solvent by evaporation, said sizing agent in such solution being characterized by being substantially unreacted upon by alkali, said sizing agent being further characterized by being capable of imparting a substantially uniform sizing effect at a temperature at which no substantial fluxing of said sizing agent occurs.

HAROLD ROBERT RAFTON.